

Feb. 2, 1954

E. D. MARTIN

2,668,130

APPARATUS AND METHOD FOR CONTINUOUS PICKLING  
AND REGENERATION OF CONTACT ACID

Filed June 25, 1947

3 Sheets-Sheet 1



Feb. 2, 1954

E. D. MARTIN

2,668,130

APPARATUS AND METHOD FOR CONTINUOUS PICKLING  
AND REGENERATION OF CONTACT ACID

Filed June 25, 1947

3 Sheets-Sheet 2



Feb. 2, 1954

E. D. MARTIN

2,668,130

APPARATUS AND METHOD FOR CONTINUOUS PICKLING  
AND REGENERATION OF CONTACT ACID

Filed June 25, 1947

3 Sheets-Sheet 3



## UNITED STATES PATENT OFFICE

2,668,130

## APPARATUS AND METHOD FOR CONTINUOUS PICKLING AND REGENERATION OF CONTACT ACID

Edwin D. Martin, Chicago, Ill., assignor, by mesne assignments, to Koppers Company, Inc., Pittsburgh, Pa., a corporation of Delaware

Application June 25, 1947, Serial No. 757,008

12 Claims. (Cl. 134—13)

**1**

The invention relates to an apparatus for and method of pickling iron and steel and for treating the spent pickle liquor so that it is regenerated and thus re-usable for pickling.

The art of pickling has long been employed in the production of iron and steel. In fact, removal of scale from the metal by pickling has been known since very early times in the industry. In the practice of this art as commonly employed at the present time, several major problems exist. Thus, in present practice, pickling requires a longer time than is desirable, because the acid content of the spent pickle liquor must be reduced to a point where disposal of the waste liquor does not involve too great an economic loss. With such reduction in acid content, lack of uniformity of pickling on all parts of the metal is also encountered. Further, the quantity of spent pickle liquor, particularly at the larger steel mills, is so great that its disposal as waste has been threatened with legislative action.

The general object of the invention is to provide a novel apparatus and method for pickling metal and for regenerating the spent pickle liquor, which result in effective pickling of the metal and which substantially eliminate the problem of disposal of spent pickle liquor.

More specifically, it is an object to provide a novel apparatus and method for such pickling and regeneration of the pickle liquor, by which the regeneration of the liquor renders it highly effective for re-use in pickling and results in the production of a by-product of value, thereby eliminating the problem of the disposal of the liquor as a waste.

Another object is to provide a novel apparatus and method for pickling metal, which result in uniformity of pickling for all portions of the metal in a minimum of time.

A further object is to provide a novel apparatus and method for regenerating the spent pickle liquor, which make it economically practicable to maintain a relatively high acid content in the liquor for all of the pickling tanks, and do not require use of the liquor to a point where, to avoid excessive cost, its acid content is low.

Another general object is to provide an apparatus and method of the foregoing character, which make economic use of the heat employed in the method, which are simple to operate in that, to a great extent, it may be automatically controlled, and which require no great amount of change in the present type of equipment for

**2**

pickling and for the most part require only standard types of equipment for regenerating the spent liquor.

Other objects and advantages will be apparent from the following description taken in connection with the accompanying drawings, in which:

Figure 1 illustrates diagrammatically the major elements of an apparatus embodying the features of the invention.

Fig. 2 is shown, as indicated, on two sheets of the drawings and is a diagrammatic illustration of such apparatus in a commercially practicable form, particularly adapted for use in a steel mill.

In pickling of iron and steel products, the process heretofore generally employed involved a solution or pickle liquor which required dumping the spent pickle liquor purely as a waste product. The acid content of such liquor when it was fresh would be in the neighborhood of 15% of sulphuric acid, but such liquor would be used until the acid content was reduced usually to the neighborhood of 5%. Below such acid content, the pickling was altogether too slow and unsatisfactory and above that point it was felt that

there was an economic waste in dumping liquor of stronger acid content. While the pickle liquor, during pickling, was maintained at a temperature above normal room temperature, since it was known that an elevated temperature increased the ability of the solution to remove the scale from the metal, there was no particular correlation between the acid content and the temperature of the liquor. In pickling of iron and steel products, the oxides of iron forming

the scale on the surface of the metal reacted with the acid in the liquor to form an iron sulphate. The sulphate formed was the ferrous sulphate heptahydrate. The heptahydrate when deposited in the pickle tanks, as frequently occurred, gave considerable trouble in removing it. Thus, it formed a hard cake which could only be removed by chipping so that the linings of the pickle tanks, which, of course, are acid resistant, would suffer from the damage resulting from the chipping operation.

The disposal of the spent liquor has also proved to involve several major problems. Thus, since there is no recovery of any useful product, the entire cost of the pickling operation had to be included in the cost of producing the steel. Furthermore, because of the large volumes of pickle liquor used at the larger steel mills, pollution of streams and lakes has resulted since such liquid waste products eventually find their way

to such bodies of water either through sewers or from direct dumping therein.

In the present instance, the pickling apparatus herein disclosed is of the type which is utilized in connection with the pickling of strip steel, such steel constituting a large part of the production of many large steel mills. Such steel, when it comes from the mills, is rolled into coils while hot, and such coiling necessarily results in a variation in the amount and character of scale produced on different parts of the strip. Thus, the edges and end portions of the strip, particularly the tail end portion, which forms the outer part of the roll, will carry a greater amount and different character of scale than the inner portions of the roll. The latter are protected from the oxidizing effect of the air and have a different rate of cooling because of the very fact that the steel is in the form of a coil, and the adjacent turns of the coil protect one another from the action of the air except for the portions mentioned.

In pickling practice heretofore employed, such variations in the scale on the strip resulted in a lack of uniformity of pickling throughout the strip, particularly with the lower acid content of the pickle liquor just before the liquor was dumped. If such strips were held in the pickle solution long enough to completely pickle the portions where scale of certain character existed, overpickling would occur in those portions where the scale was of different character so that the result was not entirely satisfactory.

The present invention provides for a correlation between the acid content of the liquor and the temperature thereof so as to obtain an optimum rate of pickling which is substantially uniform for all portions of the strip. Furthermore, it has been found that by maintaining the acid content and temperature within a given range throughout the entire pickling process, not only can all portions of the steel be pickled to substantially the same degree in the same length of time, but also that such time is substantially shorter than was heretofore deemed necessary, particularly with the lower acid contents heretofore employed. To this end, it has been found that, if the pickle liquor is maintained at an acid concentration of at least 14% to 22% by volume of 100% sulphuric acid, and preferably between 16% and 20%, and if the pickle liquor throughout all pickling tanks is maintained at a temperature within the range of 180° to 220° F., and preferably between 200° and 210° F., then such uniformity of pickling of all parts of the metal in a relatively short period of time is attained.

Coupled with a pickling system controlled as to acid content and temperature as stated above, I provide regeneration apparatus to obtain from the spent pickle liquor a sulphate in a form which is commercially valuable, namely, ferrous sulphate monohydrate. To do so, I maintain the liquor during the recovery process at an elevated temperature, which may be substantially the same as that of the pickling bath so that there is a direct saving in heat throughout the entire apparatus. In other words, there is no intentional cooling of the liquor at any point in the system. While, of course, heat has to be added to the liquid at some point to maintain such temperatures, since they are above normal air temperature, such heat is held to a minimum by virtue of other factors, such as preheating of the metal and use of warm water for washing or rinsing purposes so that the apparatus in its entirety, while main-

taining the desired temperatures for the liquor throughout, necessitates supplying a minimum of heat to maintain such temperatures. The warm water used in rinsing is also utilized at other points in the system so that any acid and sulphate removed by the rinse water is retained in the system.

Another important feature of the invention lies in the fact that it has been found that at the above-mentioned temperatures and acid strength of the pickle solution, the presence of sulphate in the pickle liquor does not detrimentally affect or slow up the pickling operation. Preferably, the sulphate concentration in the pickle tanks is kept below the saturation point of the sulphate so that no difficulty arises from having to remove deposits of the sulphate therefrom. Because of the complete re-use of the pickle liquor and the consequent elimination of any loss of acid, the acid added to the pickle solution during regeneration need only be chemically equivalent to the amount of sulphate produced during pickling.

As mentioned above, the ferrous sulphate produced is in the form of the monohydrate rather than the heptahydrate. This chiefly results from the use of the acid concentration and the temperatures maintained both in the pickling and recovery portions of the process. While I have stated the preferred range of such temperatures, reference in the specification and claims to temperatures as being "in the neighborhood of 200° F." is intended to cover the broad range heretofore mentioned. Production of the monohydrate is obtained by precipitation thereof effected both by concentration of the spent pickle liquor with heat and by adding make-up acid to the liquor before such concentration, it being known that an increase in acid content of a pickle solution lowers the point of saturation for the sulphate. The addition of acid at this stage in the recovery process also has another benefit resulting from the fact that acid added to the solution produces heat. The monohydrate is a product which is commercially valuable and has a number of uses. Thus, the monohydrate may be used as an ingredient of fertilizer, it may be readily used in the manufacture of sulphuric acid, it is readily usable in making iron oxide pigments, it can be used in the production of iron powder for powder metallurgy, or it may be fed back into a sintering plant for use in a blast furnace. With all these uses, it has a substantial monetary value and where, in the old systems, the spent pickle liquor was all waste, the present apparatus results in no waste whatever.

Production of the monohydrate rather than the heptahydrate also provides attainment of certain other advantages. While it is preferable that the liquor in the pickle tanks be kept at a point below the saturation point of the sulphate so that no deposit of the sulphate occurs in the pickle tanks, no difficulty arises even if such deposit does occur since the monohydrate is easily broken up and, in fact, can be dissolved and washed away merely by the use of a warm water wash. The point of maximum solubility of the sulphate is at about 150° F. Consequently, by maintaining the liquor in the neighborhood of 200° throughout the entire system, as stated above, any cooling of the liquor that occurs in piping in the system merely increases the solubility of the sulphate so as to insure no deposits in such piping. It is believed that the high temperature pickling, that is, pickling at the temperatures mentioned above, together with the acid concentration tends to result in pro-

duction of the monohydrate rather than the heptahydrate. However, if the spent pickle liquor were cooled at any point in the recovery process below the temperature of 150° F. with not too high an acid concentration, the sulphate would take up water from the solution and the heptahydrate would be produced. In the present system, however, the use of temperatures in the neighborhood of 200° with the above-mentioned acid concentration not only in the pickle tanks but also throughout the entire regeneration process results in precipitation of the sulphate in the form of the monohydrate, and by removing the sulphate in this form and drying it before cooling, it will not revert to the heptahydrate form.

The apparatus illustrated in the drawings, particularly in Fig. 1, may be arranged so that a gravity feed of the liquor is utilized both throughout the pickling process and through the regeneration part. This simplifies the handling of the liquor since it need be pumped only at one point in the entire system. It has also been discovered that preheating of the metal prior to the pickling, to a temperature substantially above that of the pickle liquor, causes an action to take place when the metal is first immersed in the pickle liquor, that greatly facilitates the breaking up of the scale, so that the usual mechanical scale breaker heretofore frequently employed is no longer necessary. The pickling process also involves a treatment of the metal at an intermediate point in the pickling by a water spray to assist in the removal of red oxide from the metal, a form of scale which has heretofore caused considerable difficulty in its removal. The movement of the metal through the pickle tanks as well as the flow of liquor from one to another is concurrent and is believed to be the most satisfactory in obtaining uniform pickling and has certain engineering advantages.

As heretofore mentioned, the apparatus shown diagrammatically in Fig. 1 includes only the major elements thereof and particularly illustrates how the gravity feed of the pickle liquor may be utilized, not only in the pickling tanks, but also in the various parts of the regeneration process, with a pump placed at only one point in the entire system so that liquor will be fed by gravity through the complete circuit and back to the intake of the pump. In this figure, I have shown a plurality of pickle tanks, indicated respectively at 10, 11, 12 and 13. Four such pickle tanks have been shown for the reason that it has been found that this number of tanks is most convenient in pickling materials such as strip steel and is the number commonly employed. The steel which comes from the mill, as heretofore mentioned, is in rolls or coils, but such coils are unrolled and the strip passed continuously through the four pickle tanks, the rear end of each strip being connected to the lead end of the next strip by some means such as a seam weld which may be easily disposed of, if desired, by cutting out the seam after the pickling is completed. The flow of pickle liquor is concurrent with the movement of the steel through the pickle tanks and, to this end, pickle liquor is introduced into the tank 10 by means of an inlet pipe 14. The liquor flows from one tank to the next by connections 15 so that gravity thereby produces the flow of the liquor.

From the last tank 13, the liquor is withdrawn, and in this instance I place a pump 16 adjacent the last tank 13 to withdraw liquor therefrom as through a pipe 17. The pump 16 raises the

level of the liquor as the latter enters the regenerative part of the apparatus so that gravity flow throughout the system is thereby attained.

Treatment of the spent liquor in the regenerative portion of the apparatus comprises generally mixing of fresh acid with the spent liquor, concentration of the liquor by evaporation to cause precipitation of the ferrous sulphate, settling of the liquor to separate the precipitate from the remaining liquor, and then dilution of the separated and concentrated liquor to the desired strength for pickling. The precipitated sulphate is removed when separated from the major portion of the remaining liquor and is passed to a filter, is washed and then dried. The liquor removed in the filter together with the wash water is conducted to the point where the liquor is diluted and, with the addition of water, the regenerated liquor is returned to the initial pickle tank 10 through the inlet pipe 14. The regeneration apparatus may of course serve one or more pickling operations.

To disclose the regenerative process in somewhat more detail, in the embodiment shown in Fig. 1, the pump 16 discharges the spent liquor through a pipe 20 into a mixing tank 21 into which acid is also introduced through a pipe indicated at 22. The amount of acid added through the pipe 22, as heretofore stated, need only be the chemical equivalent of the amount of sulphate produced during the pickling operation in the tanks 10, 11, 12 and 13. The introduction of the acid at this point has a number of advantages, among which is the fact that heat is added to the liquor by the reaction of the acid therewith. Furthermore, introduction of the acid at this point in the regenerative process lowers the saturation point for the sulphate and, consequently, tends to produce precipitation of sulphate crystals.

The mixing tank 21 is connected to a second tank 23 as by a siphon 24 where evaporation of a portion of the water content of the liquor is effected. Such evaporation may be accomplished by the application of heat, although no specific means therefor is shown in the drawings. Concentration of the liquor as a result of such evaporation brings the liquor above the saturation point for the sulphate so that crystallization of the sulphate rapidly occurs in the tank 23. By constantly feeding the liquor from the mixing tank 21 to the crystallizing tank 23, a constant seeding of crystals occurs so that the crystal size may, therefore, readily be controlled. The heat applied in the crystallizing tank 24 is also sufficient to maintain the desired temperature of the liquor for pickling. Such temperature, as heretofore stated, may range from 180° to 220° F. and preferably is between 200° and 210° F.

From the crystallizing tank 23 the liquor together with the major portion of the sulphate crystals carried therein is discharged into a settling tank 25, preferably by means of a siphon 26. In the settling tank, the sulphate crystals settle to the bottom of the tank in the form of a slurry for withdrawal and further treatment, while the remaining liquor is decanted, as by means of an overflow pipe 27, to a dilution tank 30 where the liquor is diluted to the desired acid content for re-use in pickling.

The slurry containing the sulphate crystals, collecting in the bottom of the settling tank 25, is withdrawn through a pipe 31 and is discharged into a filter 32. Any sulphate crystals collecting in the bottom of the crystallizing tank 23 or mix-

ing tank 21 may likewise be discharged through the pipe 31 to the filter 32. The filter 32 is of a type which provides for separation of the solid and liquid portions of the slurry, and which also provides for washing of the solids and drying thereof. While several different types of standard filters may be used, the filter shown at 32 diagrammatically represents a rotary suction type of filter. Thus, the slurry introduced into the filter by means of the pipe 31 is first separated into crystals, which form the solid part of the slurry, and liquor. The crystals are then flash-washed by cold water introduced into the filter through a pipe 33. The wash water and the filtered liquor are discharged from the filter through a pipe 34 and are pumped to the dilution tank 30 by means of a pump 35, if necessary, through a pipe 36. Cold water is employed in such wash, since the monohydrate is more slowly soluble therein.

Because of the concentration of the liquor in the crystallizing tank 23, it of course must be diluted before it may again be used as a pickling solution. While the wash water coming through the filter 32 to some extent dilutes it, additional water as needed may be introduced into the dilution tank 30 through a pipe 37. The level of liquid in the entire system may be easily controlled by a float 40 in the dilution tank. The diluted liquor, ready for re-use in the pickling portion of the apparatus, may be discharged to the first pickle tank 10 through the pipe 14 connected to a siphon in the dilution tank 30. An overflow pipe 41 may also be provided from the dilution tank 30.

The sulphate separated from the liquor in the filter 32, after being washed by the water introduced into the filter, is quickly dried by the introduction into the filter of hot air through an inlet 38. By thus removing the moisture from the sulphate in the monohydrate form, there is no water present for the sulphate to revert to the heptahydrate. The sulphate thus remains in the monohydrate form after removal through a discharge 42, and can be easily handled without caking, where any reversion to the heptahydrate would result in caking and consequent difficulty in handling the material. The washing also eliminates any trace of acid and its consequent hygroscopic action so that the monohydrate, which is non-hygroscopic, will not absorb moisture from the air.

As heretofore mentioned, the temperature of the liquor is maintained throughout the system in the neighborhood of 200° F. The heat for this purpose is derived chiefly from the heat supplied to the crystallizing tank 23 to evaporate a portion of the water content of the liquor. Some heat is also supplied by mixing the acid with the liquor in the mixing tank 21. The total heat is sufficient to maintain the temperature in this neighborhood. While the temperature may range from 180° to 220° F., the preferred range for the liquor in entering the first pickle tank is from 200° to 210° F. Some cooling of the liquor, of course, occurs while the liquor passes through the various tanks, but preferably the flow is at such rate that the drop in temperature is not more than 10° F. between the first and last pickle tanks. The spent liquor, in entering the mixing tank 21, of course, is immediately heated to some extent by the addition of acid, and the addition of heat for evaporation purposes in the crystallizing tank 23 obviously must raise the temperature somewhat above the preferred range for

pickling to account for heat losses elsewhere. The temperature of the liquor in the regeneration portion of the apparatus, however, may be said to be within the neighborhood of 200° F. The slightly higher temperature in the regeneration portion of the apparatus is, however, beneficial since the insolubility of the sulphate decreases with an increase in temperature and, consequently, the higher temperature aids in the precipitation of the sulphate crystals. Because of the temperature maintained both in the regeneration portion of the apparatus and in the pickle tanks and because of the acid concentration, the sulphate is produced in the monohydrate form rather than the heptahydrate.

The apparatus shown in Fig. 2, disclosed on two sheets of the drawings, embodies all of the elements shown in Fig. 1. Fig. 2, however, shows the apparatus in a commercial practicable form particularly adapted for use in a steel mill in connection with pickling of strip steel. While the various elements of the apparatus included in Fig. 2 are not arranged in the drawings in such a way as to illustrate the gravity flow, as they are in Fig. 1, still these elements may be so located in an actual structure that a minimum use of power for pumping the liquor is required in the operation of the apparatus shown in Fig. 2. Certain of the elements in Fig. 2 are shown in a somewhat different form from the disclosure of Fig. 1, but such differences in form are of no particular importance and have no bearing on the scope of the invention. To simplify the disclosure, the pickling apparatus disclosed in Fig. 2 is shown on one sheet, while the apparatus used in regeneration of the liquor is shown on the other sheet, the connections between the two portions being clearly indicated.

In the pickling portion of the apparatus of Fig. 2 shown on the first sheet thereof, the usual four pickle tanks are indicated at 50, 51, 52 and 53. Regenerated pickle liquor with the acid strength and temperature heretofore stated is introduced into the first tank 50 through a line 54 and the liquor flows successively through the four tanks by connections 55 connecting the tanks in series. The spent pickle liquor is removed from the last tank 53 through a pipe 56. The strip metal is adapted to be conducted through the four pickle tanks concurrently with the flow of liquor therethrough.

One of the features of the invention lies in the treatment of the metal prior to introduction into the first pickle tank 50. Introduction of the metal at room temperature would, of course, tend to lower the temperature of the pickle liquor. It is, therefore, desirable, from that standpoint, to heat the metal to a temperature equal to or above that of the liquor in the tank 50. If the metal is heated to a temperature above such liquor, then additional heat is thereby added to the liquor and such addition, of course, is of advantage. However, an additional advantage can be obtained, which facilitates the initial removal of scale from the metal, if the metal is heated to a temperature substantially above that of the pickle liquor, so that immersion of the metal in the liquor results in a quick drop in temperature tending to "craze" or crack the scale. Preferably, the metal is heated in dry condition so that no protective layer of liquid is left on the surface of the metal when it is first introduced into the pickle liquor. The rapid reduction in temperature thereby obtained on the surface of the metal results in the before-mentioned cracking of the scale which greatly

facilitates loosening thereof and speeds up the pickling. Preferably, with the pickle liquor in the neighborhood of 200° F., the metal is dry-heated to a temperature of 240° to 250° F. by a heater indicated at 57. Such temperature, of course, is above the boiling point of water and the action taking place may involve the formation of a layer of steam on the metal tending to break up the scale. The rapid contraction of the metal and scale due to the reduction in temperature may also be a factor in the action involved. However, whatever these factors are, the results obtained prove the merit of so heating the steel before introduction into the pickle liquor. Employment of such preheating of the metal eliminates the necessity of a mechanical scale breaker, although such a breaker may be used if desired.

In the manufacture of steel, the red oxide of iron may be formed and included on the surface of the metal. Such red oxide has proved difficult to remove in ordinary pickling processes. In the present process, it has been found that spraying the metal with a warm water spray at some intermediate point in the passage of the metal from one pickle tank to another is helpful in effecting removal of the red oxide. Preferably, such warm water spray occurs at a point between the first and second pickle tanks 59 and 51. In the present instance, such spray is indicated at 60 and the warm water drains off the metal into the first pickle tank 50. While introduction of such water would have a tendency to dilute the pickle liquor, the quantity thereof is relatively small so that it does not cause any great amount of dilution. The temperature of the water introduced by the spray 69 is preferably the same as or above the temperature of the pickle liquor so as to prevent any cooling of the latter.

Another feature of the invention lies in the treatment of the metal when it emerges from the last pickle tank 53. Such metal, of course, carries some pickle liquor with it as the metal is removed from the pickle tank and the liquor should, of course, be washed from the metal because of the acid content of the liquor. In the present apparatus, the metal is washed with warm water which is later used in the regeneration portion of the apparatus to dilute the regenerated liquor. Thus, all acid and sulphate removed from the metal by the wash water is retained in the system. The use of warm water for washing purposes also is another factor in conservation of heat in the apparatus.

Specifically, the washing of the metal is divided into two parts to insure obtaining metal which is completely free of acid and sulphate. To this end, the metal, when it first emerges from the last pickle tank 53, passes under a spray 61 which sprays warm water on the surface of the metal and thus washes off the major portion of the adherent liquor. The spray water is collected in a tank 62 and is carried away by an outlet pipe 63. The metal, after passing under the spray 61, then is immersed in warm water in a tank 64 to complete the washing or rinsing. By removal of the major portion of the liquor with the spray, the water in the immersion tank 64 is maintained at a relatively low acid and sulphate content so that the metal when withdrawn from the rinse tank 64 may be said to be completely freed of liquor. The water supplied by the spray 61 and the water in the rinse tank 64 is maintained at a temperature in the neighborhood of the metal, which, of course, is substantially the temperature of the pickle liquor, so that the metal, when it emerges from the rinse

70  
75  
80  
85  
90  
95  
100

tank 64, quickly dries in the air because of the difference in temperature between the metal and the surrounding air. The water in the rinse tank 64 is constantly being replaced, an inlet 65 being provided for fresh water and the water being drained from the tank 64 through a connection 68 with the spray 61.

The spent liquor removed from the last pickle tank 53 through the pipe 56 is conducted to the regeneration portion of the apparatus shown on the second sheet of drawings for this figure. Inlets 70 may be provided in the line 56 to introduce water therein for flushing purposes when necessary. The line 56 conducts the liquor to a surge tank 71, from which it is withdrawn by means of a pump 72 for discharge into a filter 73. The filter 73 removes any solids, such as scale, carried over from the pickle tanks by the line 56.

From the filter 73, the liquor is conducted by a line 74 to a mixing tank 75 in which sulphuric acid is added to the liquor. Thus, an acid storage tank 76 is provided and a pump 77, of suitable construction for handling acid, feeds acid into the mixing tank 75 where the acid is thoroughly mixed with the spent liquor. Mixture of the acid with the liquor at this point in the regeneration process has several advantages, as heretofore mentioned. Thus, it creates heat in the liquor and reduces the point of saturation of the sulphate, facilitating precipitation of the sulphate at later stages in the regeneration process. Since no liquor is lost from the system, the quantity of sulphuric acid added in the mixing tank is just sufficient to make up for the amount of sulphate formed during the pickling process. As heretofore mentioned, the acid added is sufficient to establish an acid strength of 14% to 22% by volume of 100% sulphuric acid, and preferably 16% to 20%, when the liquor enters the first pickle tank.

From the mixing tank 75, the liquor with its increased acid content is forced by a pump 80 through a line 81 to a point in the apparatus where the liquor is concentrated by the evaporation of some of the water content thereof. In the present instance, such evaporation is effected by discharging the liquor through a spray 82 located in a stream of hot gas. The hot gas may be supplied from a suitable furnace 83, shown in the drawings as being provided with a gas booster pump 84 and an air blower 85. The furnace 83 in the present instance is shown as a gas-burning type since coke oven gas is readily available at most steel mills and, therefore, is an economical fuel to employ. The hot gases generated in the furnace 83 are conducted to the point where the liquor is introduced through the spray 82, by means of a flue 86. In the specific apparatus herein shown, it is contemplated that the flue gases passing through the flue 86 will have a temperature in the neighborhood of 2000° F. To regulate the temperature of the flue gases to any point desired, an air by-pass 87 may be provided for introducing air from the blower 85 directly into the flue 86. The heat obtained from the gases is not only sufficient for evaporation, but also raises the temperature of the concentrated liquor so that its eventual return to the pickle tanks will be at the desired temperature.

From the spray 82, the liquor together with the flue gases may be conducted to a centrifugal evaporator 90 to separate the concentrated liquor from the flue gas carrying the evaporated moisture. Additional liquor may be introduced into the centrifugal evaporator 90 by means of sprays

so as to obtain the greatest benefit of the heat of the gases. The moisture-carrying gases are then conducted through a passage 92 to a point where the rinse water collected in the outlet pipe 63 from the rinse tanks 62 and 64 of the pickling apparatus is introduced into such gases by means of a spray 93 to lower the temperature thereof and condense a major portion of the entrained moisture. The rinse water together with the condensate and cooled gases are then conducted to an entrainment separator 94. The latter separates the gas from the liquid and the former is carried through a passage 95 to a precipitator 96 in which any acid remaining in the gas is removed. The acid, if of sufficient quantity, may be conducted to the mixing tank 75 through a line 97.

The concentrated liquor separated from the moisture-laden gases in the centrifugal evaporator 90 is drained therefrom through a pipe 100 into a settling tank 101 where the crystallized sulphate separates, in the form of a slurry, from the supernatant liquor. In order to prevent turbulence in the contents of the settling tank 101, the pipe 100 discharges the concentrated liquor into a spillway 102 within the settling tank and the liquor overflows the top of the spillway into the main contents of the tank without stirring up the contents thereof. In the settling tank 101, the bulk of the settling of the sulphate crystals occurs within a few minutes. However, the capacity of the tank is such as to cause a relatively slow flow therethrough so that liquor may be permitted to settle up to two hours to thoroughly separate the crystals from the supernatant liquor. The presence of sulphate crystals in the liquor in the settling tank has a seeding effect to control the crystal size. The temperature of the liquor in the settling tank is somewhat higher than the liquor as it is withdrawn from the pickling tanks because of the heat added from the furnace 83. Such higher temperature, while in the neighborhood of 200° F., of course, is beneficial in increasing the precipitation of the sulphate since the saturation point for the sulphate above a temperature of, say, 150° F., decreases. The elevated temperature of the liquor in the settling tank 101 also produces a moisture-laden atmosphere in the top thereof, and such atmosphere may be conducted through a pipe 103 to the passage 92 which carries off the moisture-laden gases from the centrifugal evaporator 90. To insure maintenance of the liquor in the tank 101 at the desired temperature, heat is preferably supplied to the liquor while in the settling tank. Thus, hot gases may be introduced into the liquor in the settling tank by a line 104 extending from the furnace 83. The liquor therein may also be heated by steam coils 107 within or encasing the tank 101 and supplied with superheated steam. The steam, of course, may be drawn from an outside source or may be generated in the furnace 83, a water or wet-steam inlet 108 being shown for the latter purpose.

The liquor in the settling tank may also be recirculated through the spray 82 and the centrifugal evaporator 90 to secure greater concentration and to obtain seeding of crystals, if desired. To this end, a pipe 105 extends from the tank 101 with inlets either from the main portion of the tank or from the spillway 102, and a pump 106 connected to the pipe 105 and to the line 81 which conducts the liquor to the spray 82 will thus recirculate the liquor through the latter.

The supernatant liquor resulting from the settling in the tank 101 is withdrawn therefrom for dilution and re-use in the pickling tanks. To this end, the relatively clear supernatant liquor is decanted from the settling tank 101 through a pipe 110 and is conducted thereby to a dilution tank 111. Water for diluting the concentrated liquor in the dilution tank 111 is preferably the water and condensate draining from the entrainment separator 94, a drain pipe 112 being provided for this purpose. Such water, as heretofore stated, is the rinse water that has been employed in the rinse tanks 62 and 64 and has functioned to condense the vapor carried over into the entrainment separator from the centrifugal evaporator 90. The water thus supplied through the pipe 112 is at the desired temperature so that no loss of heat occurs. The water passing through the pipe 112, of course, carries some acid and sulphate as a result of its function of rinsing the metal, but the content thereof is so low that the water serves to dilute the concentrated liquor withdrawn from the settling tank 101. Such dilution is controlled so that the diluted liquor has the proper acid content and is reduced sufficiently in sulphate content to permit re-use in pickling. To provide for such re-use, the supply pipe 54 which feeds the regenerated liquor to the first pickle tank 50 is connected to the dilution tank 111 to receive liquor therefrom.

The sulphate precipitated by evaporation in the centrifugal evaporator 90 and precipitated in the settling tank 101, of course, is the monohydrate because of the temperature and acidity at which such precipitation occurs. The slurry containing the crystals of the monohydrate collects in the bottom of the settling tank 101 and is discharged through a drain 113 at the bottom thereof to a filter 114. In this instance, the filter is illustrated as of the rotary disk type. In the filter 114, the remaining liquor in the slurry is separated from the monohydrate crystals and is drained therefrom through the drain 115. In order to insure complete removal of the liquor and acid from the crystals, the latter are washed with cold water supplied by a pipe 116 in the filter. The acid, if any were permitted to remain on the crystals, would have a hygroscopic action. By washing the crystals, substantially all such acid is removed and the monohydrate, which is non-hygroscopic, will not absorb any moisture from the air. The wash water used at this point in the system is cold, that is, substantially at room temperature, because of the fact that the monohydrate is slowly soluble in water at this temperature. The wash water mixes with the liquor filtered from the slurry and passes out through the drain 115 along with the liquor. The washed sulphate is constantly removed from this filter 114 and is discharged into a dryer indicated generally at 117, into which hot air is introduced, as at 120, to quickly dry the sulphate. This prevents any moisture from the wash water from forming the heptahydrate and, consequently, no hard caking of the sulphate occurs in the dryer, and the sulphate in the monohydrate form can, therefore, be readily handled.

The liquor and wash water carried by the drain 115 is discharged into a receiver 121 from which it may be withdrawn by a pump 122 and carried to the dilution tank 111 through a pipe 123. The amount of cold water employed in washing the sulphate crystals in the filter is so small that it will have no material tendency to lower the tem-

perature of the liquor in the dilution tank 111. Vapor occurring in the receiver 121 may be carried through an exhaust pipe 124 to a condenser 125 with the condensate derived therefrom discharged by the pump 122 into the dilution tank 111. Moisture-laden air from the condenser may be carried over into a vacuum type moisture trap 126, and the liquid collected therein is similarly drained by the pump 122 and discharged into the dilution tank 111.

From the foregoing description, it will be apparent that the apparatus and process herein described result in effective pickling of the metal and eliminate the problem heretofore existing of disposal of spent pickle liquor. By maintaining the temperature of the liquor substantially in the neighborhood of 200° F. with the desired acid concentration throughout the entire system, that is, both in the pickling portion of the apparatus and in the regeneration portion thereof, the desired character of pickling is attained, and in the regeneration of the liquor a valuable by-product is produced. In addition to maintaining the temperature at the desired point, the acid content of the liquor is also controlled so that all parts of the metal are uniformly pickled in substantially the same time, which time is reduced to a minimum by the present process. By maintaining the temperature and acid content of the pickle liquor at the desired values, the presence of sulphate in the pickle liquor has no detrimental effect on the pickling operation. Consequently, the regeneration process need only reduce the sulphate content of the pickle liquor to such extent that the increase in sulphate content in the pickle tanks will not raise it above the saturation point. There is no intentional cooling of the liquor at any point in the process so that conservation of heat is a characteristic of the system and the system is, therefore, economical to operate in this respect. Furthermore, the re-use of the liquor and the saving of all sulphate derived in the system permit, from an economical standpoint, the use of a higher acid content for the liquor than has heretofore been deemed practicable.

I claim:

1. A continuous cyclic process for the pickling of iron and steel and for regenerating the used pickle liquor which comprises conducting the pickling operation with a pickle liquor having an acid concentration maintained within the range of from about 14% to about 22% by volume of sulfuric acid and maintaining the liquor at a temperature of from about 180° F. to about 220° F. whereby to permit rapid and uniform pickling at a relatively high ferrous sulfate concentration; continuously withdrawing used pickle liquor from the pickling step for regeneration and continuously concentrating the used liquor by evaporation; continuously adding fresh sulfuric acid to the pickle liquor being regenerated while at the same time maintaining the concentrated liquor at a temperature of from about 180° F. to about 220° F. whereby to effect rapid crystallization and precipitation of ferrous sulfate solely in the monohydrate form as a result of the combined effects of said temperature and increased acidity in lowering the solubility of ferrous sulfate monohydrate; continuously separating crystallized and precipitated ferrous sulfate monohydrate and thus obtaining a resultant concentrated liquor having a sulfuric acid concentration above said range; continuously diluting said resultant concentrated liquor

with sufficient water to obtain a regenerated pickle liquor having an acid concentration within said range; maintaining the pickle liquor at all times throughout the aforementioned regeneration steps at a temperature of from about 180° F. to about 220° F. whereby to provide a regenerated pickle liquor adapted for continuous recirculation to the pickling step without reheating; and continuously recirculating the regenerated pickle liquor directly to the pickling step whereby to provide a continuous pickling and regeneration system characterized by high heat economy and low heat input requirements as a result of the maintenance of substantially the same operating temperature during both pickling and regeneration.

2. The process of claim 1 further characterized in that said acid concentration in the pickling step is within the range of from about 16% to about 20% by volume of sulfuric acid.

3. A continuous cyclic process for the pickling of ferrous metal and for regenerating the used pickle liquor which comprises pickling the metal with a pickle liquor having an acid concentration maintained within the range of from about 14% to about 22% by volume of sulfuric acid and maintaining the liquor at a temperature of from about 180° F. to about 220° F. whereby to permit rapid and uniform pickling at a relatively high ferrous sulfate concentration; continuously removing the metal from the pickling step and rinsing the pickled metal with warm water to remove pickle liquor therefrom; continuously withdrawing used pickle liquor from the pickling step for regeneration and continuously regenerating the same by concentrating the liquor and crystallizing and precipitating ferrous sulfate monohydrate therefrom while maintaining the liquor at a temperature of from about 180° F. to about 220° F.; continuously adding fresh sulfuric acid to the pickle liquor during regeneration; continuously separating concentrated liquor from the precipitated ferrous sulfate monohydrate; continuously diluting said concentrated liquor with water including the effluent warm rinse water from the rinsing step whereby to obtain a regenerated pickle liquor having an acid concentration within said range and having a temperature of from about 180° F. to about 220° F.; and continuously recirculating the diluted pickle liquor to the pickling step without reheating thereby providing a continuous pickling and regeneration system wherein the heat of the rinse water assists in maintaining the temperature of the regenerated liquor during dilution thereof whereby to maintain the liquor at a temperature of from about 180° F. to about 220° F. substantially throughout the entire process.

4. A continuous cyclic process for the pickling of ferrous metal and for regenerating the used pickle liquor which comprises pickling the metal with a pickle liquor having an acid concentration maintained within the range of from about 14% to about 22% by volume of sulfuric acid and maintaining the liquor at a temperature of from about 180° F. to about 220° F. whereby to permit rapid and uniform pickling at a relatively high ferrous sulfate concentration; continuously removing the metal from the pickling step and rinsing the pickled metal with warm water to remove pickle liquor therefrom; continuously withdrawing used pickle liquor from the pickling step for regeneration and continuously regenerating the same by contacting the used liquor

with hot gases whereby to concentrate the liquor by evaporation of water therefrom; continuously separating a concentrated liquor from effluent gases; continuously scrubbing said effluent gases with the effluent warm rinse water from the rinsing step; crystallizing and precipitating ferrous sulfate monohydrate from the concentrated liquor while maintaining the liquor at a temperature of from about 180° F. to about 220° F.; continuously adding fresh sulfuric acid to the 10 pickle liquor during regeneration; continuously separating concentrated liquor from the precipitated ferrous sulfate monohydrate; continuously diluting said concentrated liquor with water including the effluent warm rinse water from the scrubbing step whereby to obtain a regenerated pickle liquor having an acid concentration within said range and having a temperature of from about 180° F. to about 220° F.; and continuously recirculating the diluted pickle liquor to the pickling step without reheating thereby providing a continuous pickling and regeneration system wherein the heat of the rinse water assists in maintaining the temperature of the regenerated liquor during dilution thereof whereby to maintain the liquor at a temperature of from about 180° F. to about 220° F. substantially throughout the entire process.

5. A continuous cyclic process for the pickling of ferrous metal and for regenerating the used pickle liquor which comprises pickling the metal with a pickle liquor having an acid concentration maintained within the range of from about 14% to about 22% by volume of sulfuric acid and maintaining the liquor at a temperature of from about 180° F. to about 220° F. whereby to permit rapid and uniform pickling at a relatively high ferrous sulfate concentration; continuously removing the metal from the pickling step and rinsing the pickled metal with warm water to remove pickle liquor therefrom; continuously withdrawing used pickle liquor from the pickling step for regeneration and continuously concentrating the used liquor by evaporation and then crystallizing and precipitating ferrous sulfate monohydrate while maintaining the liquor at a temperature of from about 180° F. to about 220° F.; continuously adding fresh sulfuric acid to the pickle liquor during regeneration; continuously settling the concentrated liquor and continuously separating a clear supernatant liquor comprising a major portion of said concentrated liquor from a slurry containing said ferrous sulfate monohydrate and a minor portion of said concentrated liquor; continuously separating solid ferrous sulfate monohydrate from the liquor portion of said slurry and combining the latter with said supernatant liquor; continuously diluting the combined liquors with water including the effluent warm rinse water from the rinsing step whereby to obtain a regenerated pickle liquor having an acid concentration within said range and having a temperature of from about 180° F. to about 220° F.; and continuously recirculating the diluted pickle liquor to the pickling step without reheating thereby providing a continuous pickling and regeneration system wherein the heat of the rinse water assists in maintaining the temperature of the regenerated liquor during dilution thereof whereby to maintain the liquor at a temperature of from about 190° F. to about 220° F. substantially throughout the entire process.

6. A continuous process for regenerating used sulfuric acid pickle liquor containing ferrous

sulfate and having an acidity not less than about 14% by volume of sulfuric acid, which comprises continuously concentrating the liquor by evaporation; continuously subjecting the concentrated liquor to an elevated temperature of from about 180° F. to about 220° F. in the presence of added fresh sulfuric acid whereby to effect rapid crystallization and precipitation of ferrous sulfate solely in the monohydrate form as a result of the combined effects of increased temperature and increased acidity in lowering the solubility of ferrous sulfate monohydrate; continuously recovering the crystallized and precipitated ferrous sulfate monohydrate and separating, without further removal of ferrous sulfate, a concentrated liquor having a sulfuric acid content greater than about 22% by volume; continuously diluting the separated liquor with sufficient water to obtain a regenerated pickle liquor having a pickling concentration of from about 14% to about 22% by volume of sulfuric acid; and maintaining the liquor at all times throughout the aforementioned steps at a temperature within the range of from about 180° F. to about 220° F. whereby to provide a regenerated pickle liquor adapted for use in pickling without reheating.

7. The process of claim 6 further characterized in that a portion of the concentrated liquor is recycled from the crystallizing and precipitating step to the evaporating step for seeding the used liquor during evaporation thereof.

8. A continuous process for regenerating used sulfuric acid pickle liquor containing ferrous sulfate and not less than about 14% by volume of sulfuric acid which comprises continuously concentrating the used liquor to an acid concentration greater than about 22% by volume by evaporation and the addition of fresh sulfuric acid; continuously maintaining the concentrated liquor at a temperature of from about 180° F. to about 220° F. whereby to effect rapid crystallization and precipitation of ferrous sulfate solely as the monohydrate and in a crystalline form of high settling rate; continuously settling the concentrated liquor and separating a clear supernatant liquor comprising a major portion of said concentrated liquor from a slurry containing said ferrous sulfate monohydrate and a minor portion of the concentrated liquor; continuously separating ferrous sulfate monohydrate from the liquor portion of said slurry; continuously combining the latter with said supernatant liquor; and continuously diluting the combined liquors with sufficient water to obtain a regenerated pickle liquor having an acid concentration of from about 14% to about 22% by volume of sulfuric acid.

9. A continuous process for regenerating used sulfuric acid pickle liquor containing ferrous sulfate and not less than about 14% by volume of sulfuric acid which comprises continuously concentrating the used liquor to an acid concentration greater than about 22% by volume by evaporation and the addition of fresh sulfuric acid; continuously maintaining the concentrated liquor at a temperature of from about 180° F. to about 220° F. whereby to effect rapid crystallization and precipitation of ferrous sulfate solely as the monohydrate and in a crystalline form of high settling rate; continuously settling the concentrated liquor and separating a clear supernatant liquor comprising a major portion of said concentrated liquor from a slurry containing said ferrous sulfate monohydrate and a minor portion

of the concentrated liquor; continuously separating ferrous sulfate monohydrate from the liquor portion of said slurry; continuously combining the latter with said supernatant liquor; continuously washing the separated ferrous sulfate monohydrate with water; and continuously diluting the combined liquors with water including the effluent wash water from said washing step whereby to obtain a regenerated pickle liquor having an acid concentration of from about 14% to about 22% by volume of sulfuric acid.

10. In a process for regenerating used sulfuric acid pickle liquor by concentrating the liquor and precipitating crystalline ferrous sulfate monohydrate therefrom, the steps of separating the ferrous sulfate monohydrate crystals from the concentrated liquor, washing the separated crystals with water at substantially room temperature to remove adsorbed acid liquor therefrom without dissolving the crystals to any substantial extent, and immediately thereafter rapidly drying the washed crystals whereby to obtain acid-free non-hygroscopic crystals of ferrous sulfate monohydrate and whereby to avoid formation of ferrous sulfate heptahydrate and consequent caking thereof.

11. In apparatus for continuously pickling ferrous metal with sulfuric acid pickle liquor and for regenerating the used pickle liquor, the combination of a plurality of interconnected pickle tanks adapted to contain the pickle liquor, a rinse tank disposed adjacent the pickle tanks for rinsing the metal with water after pickling, an evaporator for concentrating the used pickle liquor to precipitate ferrous sulfate monohydrate therefrom, conduit means interconnecting said pickle tanks with said evaporator for supplying used pickle liquor from said pickle tanks to said evaporator, a settling tank having a direct fluid connection with the evaporator for separating the concentrated liquor from the precipitated ferrous sulfate monohydrate, a dilution tank having a conduit connecting the same with the upper portion of said settling tank for supplying supernatant concentrated liquor from the settling tank to the dilution tank, conduit means interconnecting said rinse tank and said dilution tank for supplying effluent rinse water from the rinse tank to said dilution tank and diluting the concentrated liquor with said rinse water, and conduit means interconnecting said dilution tank and said pickle tanks for recirculating the diluted liquor directly to said pickle tanks.

12. In apparatus for continuously pickling ferrous metal with sulfuric acid pickle liquor and

55

for regenerating the used pickle liquor, the combination of a plurality of interconnected pickle tanks adapted to contain the pickle liquor, a rinse tank disposed adjacent the pickle tanks for rinsing the metal with water after pickling, an evaporator for concentrating the used pickle liquor to precipitate ferrous sulfate monohydrate therefrom, means for supplying hot gases to said evaporator, conduit means interconnecting said pickle tanks with said evaporator for supplying used pickle liquor from said pickle tanks to the evaporator for contact with the hot gases, a settling tank having a direct fluid connection with the evaporator for separating the concentrated liquor from the precipitated ferrous sulfate monohydrate, a dilution tank having a conduit connecting the same with the upper portion of said settling tank for supplying supernatant concentrated liquor from the settling tank to the dilution tank, a scrubber having a fluid connection with said evaporator for receiving effluent gases from the latter, conduit means connected to said rinse tank and to said scrubber for passing effluent rinse water from the rinse tank to the scrubber for contact with the gases therein, a conduit interconnecting said scrubber and said dilution tank for supplying effluent rinse water from the scrubber to said dilution tank for diluting the concentrated liquor with said rinse water, and conduit means interconnecting said dilution tank with said pickle tanks for recirculating the diluted liquor directly to said pickle tanks.

EDWIN D. MARTIN.

35 References Cited in the file of this patent

UNITED STATES PATENTS

| Number    | Name            | Date          |
|-----------|-----------------|---------------|
| 1,045,723 | McFetridge      | Nov. 26, 1912 |
| 1,146,071 | Hoffman         | July 13, 1915 |
| 1,865,607 | Allen           | July 5, 1932  |
| 2,005,120 | Whetzel et al.  | June 18, 1935 |
| 2,017,773 | Smith et al.    | Oct. 15, 1935 |
| 2,050,355 | McCollam        | Aug. 11, 1936 |
| 2,078,088 | Mantius et al.  | Apr. 20, 1937 |
| 2,118,272 | Smith           | May 24, 1938  |
| 2,155,854 | Barnes          | Apr. 25, 1939 |
| 2,185,095 | Smith et al.    | Dec. 20, 1939 |
| 2,203,606 | Whitfield       | June 4, 1940  |
| 2,322,134 | Hodge           | June 15, 1943 |
| 2,372,599 | Nachtman        | Mar. 27, 1945 |
| 2,379,823 | Mottern         | Jan. 3, 1945  |
| 2,381,652 | Dishauzi        | Aug. 7, 1945  |
| 2,541,901 | Zademach et al. | Feb. 13, 1951 |